

# UNITED STATES PATENT OFFICE.

ERNST MURMANN, OF VIENNA, AUSTRIA-HUNGARY.

## ALUMINIUM ALLOY.

SPECIFICATION forming part of Letters Patent No. 699,216, dated May 6, 1902.

Application filed August 14, 1900. Serial No. 26,833. (No specimens.)

*To all whom it may concern:*

Be it known that I, ERNST MURMANN, a subject of the Emperor of Austria-Hungary, residing at 14 Kettenbrückengasse, Vienna, Austria-Hungary, have invented certain new and useful Improvements in Aluminium and Brass Alloys, of which the following is a specification.

This invention relates to an aluminium alloy which owing to the readiness with which it lends itself to further treatment or manipulation will prove a preëminently workable metal in those cases where no importance is attached to the alloy attaining its maximum of lightness.

In preparing the alloy brass containing either from twenty to eighty parts of copper or from eighty down to twenty parts of zinc is added to the aluminium. By this addition of brass, which should be comprised somewhere between the limits of from five to thirty-five parts to every one hundred parts of aluminium, a good workable alloy will be obtained.

With an addition of brass of from five to ten parts the alloy will be capable of being laminated and wiredrawn.

With an addition of at least ten parts of brass the alloy will reach the point at which it is workable with a file and with cutting-tools with a markedly better effect than before, while this workability will attain its maximum if the addition be raised to twenty parts, when the alloy will be hardest, but without becoming brittle. With thirty-five parts of brass the alloy will become softer again, yet without its workability being thereby materially affected. It will at the same time be more brittle, however. Where the percentage exceeds thirty-five parts, the alloy becomes noticeably heavier and more like the familiar aluminium brass or aluminium bronze.

Where it is desired to produce soft and cheap

material, the alloy is made richer in zinc and takes the form of what is termed "white brass." Where the object is to obtain a product of maximum density, an alloy is composed of from forty-five to seventy-five parts of copper and of from fifty-five to twenty-five parts of zinc. By increasing the proportion of copper beyond seventy-five to eighty parts no appreciable advantage will be secured, for beyond that limit, or, in other words, where the "tombac" added is richer than that in copper the aluminium alloys obtained will be soft, and it will be impossible neatly or finely to work same with cutting-tools, as is the case with aluminium and copper alloys.

The alloy best suited to most purposes consists of one hundred parts of aluminium, thirteen parts of copper, and seven parts of zinc, or, in other words, twenty parts of brass. An excellent alloy is yielded by a composition of forty-eight molecules of aluminium, one molecule of copper, and one molecule of zinc—that is to say, one hundred parts of aluminium, 9.81 parts of copper, and 10.1 parts of zinc.

Greater density may be imparted to the alloy by cooling it rapidly, also by superadding predetermined quantities of calcium, barium, and strontium to the alloy.

Having now described my invention, what I claim as new, and desire to secure by Letters Patent, is—

An aluminium alloy consisting of one hundred parts of aluminium to three to sixteen parts of copper to twelve to two parts of zinc, the amount of zinc being twice the amount of copper, substantially as set forth.

In testimony that I claim the foregoing as my invention I have signed my name in presence of two subscribing witnesses.

ERNST MURMANN.

Witnesses:

C. B. HURST,  
ALVESTO S. HOGUE.